

Sept. 25, 1962

I. R. DUNLAP  
UNIFIED PAPER SHEET, PROCESS OF MAKING, AND  
PRESSURE-SENSITIVE ADHESIVE TAPE  
MADE THEREFROM

3,055,496

Filed May 4, 1961

3 Sheets-Sheet 1



INVENTOR  
ISAAC R. DUNLAP

BY  
*Charles A. Harris*  
ATTORNEY

Sept. 25, 1962

I. R. DUNLAP  
UNIFIED PAPER SHEET, PROCESS OF MAKING, AND  
PRESSURE-SENSITIVE ADHESIVE TAPE  
MADE THEREFROM

3,055,496

Filed May 4, 1961

3 Sheets-Sheet 2



Sept. 25, 1962

I. R. DUNLAP  
UNIFIED PAPER SHEET, PROCESS OF MAKING, AND  
PRESSURE-SENSITIVE ADHESIVE TAPE  
MADE THEREFROM

3,055,496

Filed May 4, 1961

3 Sheets-Sheet 3

Fig. 5.



Fig. 6.



Fig. 7.



## 1

3,055,496

**UNIFIED PAPER SHEET, PROCESS OF MAKING,  
AND PRESSURE-SENSITIVE ADHESIVE TAPE  
MADE THEREFROM**

Isaac R. Dunlap, Cranbury, N.J., assignor to Johnson & Johnson, a corporation of New Jersey  
Filed May 4, 1961, Ser. No. 107,752  
21 Claims. (Cl. 206—59)

This invention relates to improved unified papers suitable for many uses, particularly to unified papers useful as backings for adhesive tapes, sandpapers and the like and in artificial leathers, and to improved pressure-sensitive adhesive tapes and other products made with the improved backings; as well as to improved methods for manufacturing such papers.

This application is a continuation-in-part of my co-pending applications Serial No. 624,144 filed November 23, 1956, and Serial No. 89,687 filed February 16, 1961, both of which have since become abandoned.

It is most important that the fibers in papers of this type be unified or held together so that the paper possesses satisfactory resistance to delamination and fiber picking and will not blister or crack when flexed. For instance, paper backed pressure-sensitive adhesive tapes commonly are made by coating one side of the backing with an adhesive and then winding the tape upon itself with the coated side facing inwardly to form a roll. If a liner is not used, or some other special precaution is not taken, when the tape is rapidly unwound, the backing will be split into plies or delaminated because the adherence of the outside of the backing to the adhesive on the inside of the tape being unwound is greater than the coherence of the fibers in the backing.

The most common method of "unifying" the paper or strengthening it against splitting, is to incorporate a "unifying agent," commonly termed an "impregnant," in the web to bond the fibers together. Various extensible polymeric materials such as rubbery polymers and mixtures thereof have been used for this purpose. Such impregnants allow the sheet to retain a major portion of the characteristic flexibility of a paper web and yet bind the fibers against delamination of the backing when a roll of pressure-sensitive tape is unwound, for example. Normally sufficient unification to prevent delamination can be attained if it is possible to incorporate sufficient impregnant in the web. Typically, the web is saturated with the impregnant to provide the necessary unification. Since the cost of the impregnant is relatively high, one disadvantage of this approach is apparent. With some tapes and certain other products, such as artificial leather, in which high delamination resistance is desirable, it may not be possible or even desirable to incorporate in the web the necessary amount of impregnant to prevent delamination. For these and other reasons, this approach to solving the problem of providing the necessary delamination resistance leaves much to be desired.

In addition to the delamination resistance, or internal strength, necessary in a paper backing for pressure-sensitive adhesive tape, for example, it is necessary that the backing also possesses the necessary strength, flexibility and elongation to enable curving the tape without tearing when applying it to a surface in a desired configuration, and sufficient flatness to lie against the surface to which it is applied. Improvements in tear strength of such paper-backed pressure-sensitive tapes can be obtained,

## 2

though to a relatively small degree, by the use of soft and more highly extensible polymeric materials in the impregnant. The use of soft polymers in flat papers also increases to some small degree the elongation which can be obtained in the finished tape. However, the overall conformability of such a flat sheet is inadequate for many applications and results in tearing of the backing. Exemplary is the application of paper-backed pressure-sensitive tapes in masking a painted surface to which will be applied to a curved painted design.

Heretofore, to obtain a tape having the necessary delamination resistance, tear strength, flexibility and elongation, it has been common to rely upon the mechanical technique of creping the paper backing prior to impregnation. Creping may be described as a stepwise disruption of the starting web by the intermittent application of force to the web while the web is free to move at right angles to the plane of the web. This results in an opening up of the web and the formation of relatively large undulations or crinkles in the web, itself. The web is "opened up" by movement of the overlying fibers of the web away from one another in spaced areas of the web to increase the size and perhaps the number of the interstices between them in these areas. It is this openness that provides sufficient saturability, or allows the incorporation of enough impregnant, to provide the necessary delamination resistance. Again, this requires a high percentage of relatively costly impregnant and consequently is disadvantageous from a cost point of view.

Moreover, while elongation may be increased by the mechanical technique of creping and normally enough improvement in saturability may be obtained to provide the necessary delamination resistance, a creped masking tape backing, for example, has some marked disadvantages such as high overall caliper, tendency of the paint to bleed under the tape at the points of undulations and to build up at the edge of the tape, limited ability to form curved lines and conform to curved surfaces, and the like.

The prior art teaches that to obtain maximum delamination resistance in conventional saturating papers, the starting web must be relatively open with the fibers spaced apart in order to be able to receive a relatively large amount, or high level, of impregnant. In fact, all authorities in the art up to as late as four years after the filing date of application Serial Number 624,144, now abandoned are agreed that for proper unification, the raw paper used in preparing unified backings should be selected from highly porous, highly absorptive bibulous papers of low bulk density approaching blotting paper in texture; and that in forming such papers or in manipulating them prior to or during unification, any operation that substantially alters the foregoing characteristics would detrimentally affect the results obtained in unification.

I have discovered that by going in the opposite direction, i.e., compacting the starting web in a particular way and impregnating it, I can obtain a unified paper sheet possessing unexpectedly improved properties. I have discovered that by compacting the web horizontally with respect to its faces while applying force acting perpendicularly to said faces to resist substantial crinkling of the web body, and impregnating or incorporating a unifying agent in the web; I can obtain a unified paper sheet possessing the following properties:

(1) Unexpectedly high delamination resistance at low cost or unexpectedly great cost savings at prior art levels of delamination resistance;

(2) Extraordinary conformability, i.e., ability to be conformed smoothly and easily to curved surfaces and other three dimensional objects and to be smoothly applied in different shapes to flat surfaces;

(3) High flexibility;

(4) Flatness;

(5) Versatility in properties directly attributable to materials used.

Unified paper sheets having the above properties are ideal as backings for pressure-sensitive tapes, particularly those used as masking tapes, for example, during the spray painting of automobiles. In such tapes, not only is their unexpectedly high delamination resistance and low cost of importance, but the extraordinary conformability of the backing combined with its flatness and tear strength permit easy application to curved and irregular surfaces and give sharply defined paint lines without feathering at the edges of the tape. Due to its flat backing and to the ease with which the tape may be applied, abrasion of the fingers of the worker applying the tape also is minimized.

Heavier weight unified papers possessing the above properties also are ideal for use in artificial leathers where their superior flexibility, soft hand, freedom from blistering or splitting and freedom from fiber picking are of great importance. Papers according to this invention also are highly desirable as sandpaper backings and when used for this purpose, provide sandpapers possessing superior flexibility, tear strength and crack resistance.

Starting webs according to this invention may be creped or uncreped and include the conventional saturating papers of the prior art. Similarly these webs may be formed from fibers which are substantially straight and possess only natural curl or they may include a substantial proportion of fibers to which a substantial amount of curl or crimp has been imparted prior to web formation. The starting web comprises cellulosic fibers oriented predominantly parallel to the web faces and flatly assembled in overlapping, crossing relation with one another. When the term "face" is used in referring to the starting web or paper according to this invention, it refers to the outline of one surface of the web, roughly as it would appear to the naked eye. If the web or paper is pictured in a horizontal position, it possesses two faces, i.e., a top face and a bottom face. The "body of the web" or "web body" is that portion of the web or paper between its two faces.

The fibers in the web are relatively long compared to the thickness of the web so that the ratio of the average length of the fibers to the caliper of the web is at least about four to one, preferably at least about ten to one. This means that, even in the most extreme cases, the overall orientation of a given fiber from end to end can only be at a slight angle to the faces of the starting web and that normally this angle is negligible.

The starting web is compacted horizontally while the cellulosic fibers in the web are plasticized with moisture and heated to a temperature sufficient to generate moisture vapor. Compacting forces are applied to the web horizontally with respect to the web faces while the web body is held or restrained against substantial crinkling in a vertical direction. In other words, forces are applied approximately perpendicular to the direction of the compacting forces to resist the tendency of the web to crinkle and maintain the web faces substantially parallel to one another. The compacting forces may be applied longitudinally, or in the machine direction of the web, or laterally in the cross machine direction.

The lowest degree of compaction, i.e., percentage of length required for utility in this invention, is not greater than about 5% with some papers. However, with most papers more exhaustive treatment may be desirable. For instance, about 10-25% compaction normally is preferred, particularly when the web is treated in one pass as will

be described more fully hereinafter. The upper limit of the degree of compaction is determined both by the nature of raw untreated paper and the application for which the unified paper is intended. In a wide diversity of raw papers intended for various applications, the upper limit of compaction desired might be as high as 40% or more and might in some cases approach the lower limit of another paper intended for a different end use.

In general increasing degrees of treatment tend to decrease the tensile strength of the raw paper. However, the physical properties of a paper prior to the incorporation of the unifying material are of secondary importance in determining the usefulness of the unified paper product. The presence of a unifying material, especially in relatively large amounts relative to the untreated fiber, usually results in marked increases in such properties as tensile, tear and elongation as well as in resistance of the sheet to delamination, or splitting.

In general the amount of impregnant incorporated into the paper web is in an amount of about 10-150 percent impregnant solids by weight of the raw paper (dry web), the minimum amount thereof, comprising in all cases, an amount sufficient to unify said web to a degree whereby the forces of adhesion of the particular adhesive coated on the backings are insufficient to cause delamination of an underlying ply of tape, for example.

Although the normal practice is to treat a water plasticized web, under certain circumstances the water may comprise only a small percentage of the web weight as it is treated. The desired content of the sheet at the time of treatment is determined both by the nature of the raw paper and the end use contemplated. In general the more dense the untreated paper the greater the water content when compressed if tensile is to be retained in the finished unified paper or tape backing. Thus, a flat paper of fairly dense structure may be most advantageously treated at a water content, limited only by the amount permitted by the equipment and process, that is, the maximum which can be held by the sheet under the conditions of compaction inherent in the process. Normally and preferably the moisture content during treatment should be about 10-20% by weight of the web. However, it may be most advantageous to treat more open sheets, such as an open kraft saturating paper, at a water content at or even below that of equilibrium between the water content of the sheet and normal testing conditions for paper, 50% R.H. at 72° F. Variations of types of paper between these two types may require, or be advantageously treated, at moisture contents varying between these extreme limits. Severe treatment under conditions of little water plasticizing tends toward higher elongation by longitudinal compression and under usual conditions a higher degree of unification of the resulting paper. Whatever its moisture content, at least one side of the web is heated during treatment to a temperature sufficient to generate moisture vapor, i.e., at least about 212° F., as will be described more fully hereinafter.

By the compacting operation there is introduced a distortion of the fibers by contracting the area in which they lie, while at the same time holding the faces of the web flat and parallel thus preventing appreciable thickening of the web. Simultaneously, a substantial pressure is maintained on the faces of the web so as to prevent creping of the web and also to force the distorted fibers into voids within the web. Upon drying, the changed orientation of the fibers is retained and the web exhibits firmness and strength from the mutual adherence of the fibers. When the web is subjected to tensile stress there is an inertia to reformation arising from the mutual adhesion of the almost continuous distribution of the fibers. However, as the tensile stress is increased, the nearly continuous structure of the fibers progressively yields and the web assumes an added width or length approximately equal to the width or length by which the paper web had been compressed. Upon still further increasing the tensile

stress, the mutual adherence of the fibers which maintains the structure of the web breaks down and the sheet ruptures.

Compaction, longitudinally or laterally, in the manner described, causes the fibers to become compressively distorted, crowded and pushed together within the body of the web. Those fibers which originally are oriented primarily in the direction of compaction are caused to collapse by taking a multiplicity of kinks, crimps or tight loops as portions of the fibers are forced closer together and into the voids within the web. These kinks, crimps or tight loops, hereinafter called "kinks" occur, not only in a plane parallel to the web faces, but also in planes perpendicular thereto so that a large proportion of fiber segments forming the kinks are oriented at an angle to the web faces.

If the starting web is relatively dense as in a flat compact paper, it will retain substantially the same density during compaction and if it is dense and moderately hydrated, for instance, fiber-to-fiber bonds will be broken so that its saturability will be increased somewhat during compaction; but if the starting web is relatively open, such as in creped saturating papers, it will be considerably densified and flattened out during compaction.

The impregnant may be incorporated in the web either before or after compaction but impregnation prior to compaction is preferred for three reasons, i.e.,

(a) Greater compaction efficiency is attainable,

(b) Impregnation may be performed in conjunction with compaction for plasticizing the fibers during compaction when an aqueous impregnant is employed, and

(c) Better paper properties are attainable with an aqueous impregnant than when the web is first compacted and then impregnated.

Greater compaction efficiency, i.e., actual degree of compaction over maximum theoretical degree of compaction times one hundred, is attainable when the web is impregnated prior to compaction, especially when compaction occurs when the web is relatively "dry" and at low levels of impregnation. Since it is highly desirable to treat the web at a low moisture content to avoid moisture removal problems, and low levels of impregnation are desired to save cost; it is apparent that improved compaction efficiency under these conditions is of great importance.

The starting web may be impregnated with an aqueous impregnant, dried to bring the moisture content to about 10-20% by weight of the web, for instance, and then compacted under the above described conditions with excellent results. In this case the moisture carried into the web with the impregnant acts to plasticize the fibers of the web.

The process of this invention also is highly advantageous because of the variety of cellulosic fibers and impregnants which may be employed. As a result, the papers of this invention are versatile in so far as their properties, which may be attributed directly to the materials employed in their manufacture are concerned. For instance, both aqueous and solvent based impregnants may be used although, when the impregnant is incorporated in the web after compaction, solvent based impregnants give better results. However, if the impregnant is incorporated prior to compaction, it makes no difference whether it is water based or solvent based. Thus, it is possible to use the well known and relatively inexpensive elastomeric aqueous latices of the prior art in the process of this invention with maximum results.

In addition, whereas relatively high modulus polymers are not acceptable as unifying agents when applied in the relatively high percentages of unified papers according to the prior art if a flexible paper is desired, such polymers may be utilized and are even highly desirable, and in fact preferred, for pressure-sensitive masking tape backings, at the lower levels of impregnation made possible by this invention. For instance, polymers in the transition re-

gion of viscoelastic behavior, and even in the upper range of this region, are advantageously employed in unifying papers for certain applications according to this invention when the impregnant incorporated is about 10-50% by weight of the dry fibers. For instance, higher values for delamination resistance and other physical characteristics are attainable with a high modulus polymer when this amount of impregnant is used. The transition region of viscoelastic behavior, referred to above, is described in some detail by Arthur V. Tobolsky, in "Stress Relaxation Studies," at page 65 in *Rheology, Theory and Application, volume II*, edited by Frederick R. Eirich and published by Academic Press Inc., New York, N.Y., in 1958. Such polymers include unplasticized polyvinyl acetate polymers and copolymers, high styrene butadiene-styrene copolymers, and the like. Polymers in this region are preferred for masking tapes according to this invention to give the tape sufficient firmness for ease in application when only about 10-30% by weight of the unifying impregnant is present.

In certain cases it may be advantageous to perform impregnation and compaction in more than two steps. For instance, if the starting web is relatively dense, flat and moderately hydrated, it first may be compacted to break some fiber-to-fiber bonds, then impregnated with an elastomeric aqueous latex, and finally compacted again, for optimum results. Or, the starting web may be impregnated with a relatively small amount of an aqueous impregnant prior to compaction, then compacted with maximum compaction efficiency due to the presence of the impregnant in the web, and finally impregnated with a maximum amount of a solvent based impregnant, for optimum results.

Other and further advantages of this invention will be apparent from the following description and claims taken together with the drawings wherein:

FIG. 1 is a diagrammatic side elevation of simple apparatus useful in performing the compacting step or steps employed in the invention;

FIG. 2 is a diagrammatic side elevation of apparatus which may also be employed in conjunction with the apparatus of FIG. 1;

FIG. 3 is a cross section of an adhesive tape utilizing, as the backing, a unified sheet treated in accordance with this invention;

FIG. 4 is a diagrammatic side elevation of somewhat different apparatus useful in performing the compacting step, or steps, according to this invention;

FIG. 5 is a greatly enlarged schematic view, partly in section and partly in elevation, of a longitudinal cross section through a flat, impregnated kraft paper, prior to compaction according to this invention, at an enlargement of approximately 400 to 1;

FIG. 6 is a similar greatly enlarged schematic view of a longitudinal cross section through a creped, impregnated saturating paper according to this invention and at the same enlargement as FIG. 5;

FIG. 7 is a schematic view similar to FIGS. 5 and 6, and at the same enlargement, of the webs of either FIGS. 5 or 6 as they would appear after being compacted according to this invention.

The apparatus of FIG. 1 comprises rolls 10, 11, 12 and a heated driven roll, or drum, 13 and a thick belt 15 with a contractile surface layer preferably of rubber of durometer hardness sufficient to prevent creping of the paper web. This belt may be formed of natural rubber or rubber substitutes, a relatively inextensible layer faced with a readily extensible and contractile surface layer of any suitable material of smooth contractile surface of sufficient hardness and extensibility, rolls 10 and 13 being adjustably movable toward or from each other so as to properly nip the belt 15 between them where the belt passes from roll 10 to the drum 13, and roll 12 being spaced away from the drum 13 sufficiently to give the belt a short straight run from the drum 13 to roll 12. As the

belt passes from roll 10 to the drum 13, the outer surface of the rubber belt which is convexly curved on roll 10 becomes concavely curved on the drum 13 and accordingly shortens. A paper web, which has been impregnated with a water base impregnant, fed in between the belt and the drum 13 where this shortening of the belt surface is taking place, is forced into such frictional contact with the contracting surface of the belt that the belt surface tends to compact, or compress, the web, parallel with the surfaces of the web. While the apparatus shown is intended to compact the web in the machine direction of the web, the web may be compacted laterally, i.e. transversely of the direction in which it was made on the paper machine, by turning short lengths sidewise and passing them individually through the apparatus. The drum 13 must be accurately machine ground and finished to a true cylinder of smooth periphery. It is heated not only to cause a partial drying of the web but also to lower the coefficient of friction between the drum and the moist web while at the same time heating the contained water and thus cause a softening and increased flexibility of the fibers. The resulting loss of water in the web makes room between the fibers for further compaction of the web as may be desired. The coefficient of friction between the wet web and the heated drum 13 is most effectively reduced at drum temperatures about 212° F. The coefficient of friction of the surface of the drum 13 is relatively low as compared to the coefficient of friction of the web-containing surface of the belt 15, so that under the influence of the contracting belt surface the paper web tends to partake of such contraction of the belt surface and slide with relation to the roll surface. During the lateral or longitudinal compaction of the paper, the tension in the rubber belt is maintained sufficiently high so that with the selected hardness of the belt surface the pressure between the rubber belt 15 and the drum 13 prevents the paper from creping and keeps the surfaces of the paper substantially flat and parallel, so that as the web is compressively shortened, individual fibers of the paper which lie generally crosswise or lengthwise of the web or in the direction of shortening are compressively distorted crosswise or lengthwise within the body of the web. Rubber is preferred as the material for the contracting surface, such as that of the belt 15, because of its ability to withstand strong tension and heavy pressure transverse to its surface, thus enabling a relatively large and effective contraction of this surface to take place without allowing the paper to crepe in response to such contraction. Rubber is also preferred for its continuously smooth surface and for its ability to grip the paper frictionally to the extent of compacting the paper laterally or longitudinally in the presence of the heavy pressure exerted between the belt and the drum 13 for prevention of creping. In the apparatus as shown, it is preferable that the rubber is reinforced by comparatively inextensible material such as heavy canvas or layers of strong cords so that the necessary high tension in the belt may be maintained and also so that the surface of the belt will expand and contract uniformly while passing over the roller 10 and the heated driving drum 13.

The apparatus of FIG. 2 was employed in conjunction with the apparatus of FIG. 1 principally to facilitate drying of the paper web. As shown in FIG. 2, a moisture-permeable belt 21 passes over an intake roll 21a and thence onto and around a heated drum 20, holding the paper web against the drum during drying.

Certain other mechanisms and procedures useful for carrying out the compression procedure employed in producing the backings of the present invention are shown and described in United States Patent No. 2,021,975 and Australian Patent No. 160,684.

Referring to FIG. 4 of the drawings there is shown apparatus similar to that of FIG. 1 which comprises; a heated metal drum 31 having a smooth, inelastic substantially unyieldable surface 32, a nip roll 33 and a relatively

thick continuous rubber compacting belt 34 passing over the nip roll 33 and between the nip roll and the heated drum 31. The compacting belt 34 is similar to the belt shown in FIG. 1 and presents a contractile, yieldably supported rubber outer surface 35 toward the drum. After it leaves the nip roll 33, the belt wraps around a portion of the drum surface 32, say about a 90° segment thereof, leaves the surface of the drum to pass around a tensioning roll 36 spaced to the left of the drum in FIG. 4, and then passes down from the tensioning roll 36 around a bottom guide roll 37 and finally back up to the nip roll 33. The amount that the belt 34 wraps around the drum 31 can be considerably less than a 90° segment of the drum surface or it can be considerably more as evidenced by the approximately 180° wrap shown in FIG. 1.

The nip roll 33 is adjustable toward and away from the surface of the drum 31 to control pressure upon the belt 34 passing between the nip roll and the drum and thereby regulate the pressure between the drum 31 and the belt 34 at the nip 38. The tensioning roll 36 is considerably spaced from the drum so that the belt passes from the drum to the tensioning roll in a long straight run 39. The tensioning roll 36 also is adjustable toward and away from the drum 31 to regulate the tension on the continuous compacting belt 34 and thereby regulate the pressure between the drum and the belt after the belt leaves the nip 38.

A starting web 40, which may have a suitable impregnant or unifying material already incorporated therein, is unwound from the supply roll 41 at the right of FIG. 4 and led into a steam chest 42 wherein it is exposed to saturated steam for a period of approximately 30 seconds to plasticize the web and adjust its moisture content to about 10-20%, preferably about 15-20% by weight of the dry web. The moistened web 40 is led from the steam chest over an exit roller 43 up and over a pair of guide rollers 44 and 45 and then down into the nip 38 formed between the drum 31 and the belt 34 where the belt passes over the nip roll 33.

As the belt 34 passes over the nip roll 33, its outer surface 35 follows a convex path while its inner surface follows a concave path with respect to the axis of curvature of the belt with the result that its outer surface 35 is stretched, or expanded, as at C in FIG. 4. Correspondingly, as the belt 34 passes the nip 38 and begins to follow the surface 32 of the drum 31 instead of the surface of the nip roll 33, its outer surface 35 begins to follow a concave path and accordingly shortens, or contracts, as at V in FIG. 4. The belt is compressed somewhat at the nip 38 so that it normally contacts the drum 31 at a point spaced above the plane P—P common to the axes of the drum and the nip roll while its outer surface 35 still is expanded in its convex path over the nip roll 33. Thus, the outer surface 35 of the belt 34 is expanded where it first contacts the web 40 and where the web 40 first is gripped between the belt 34 and the drum 31. In the area where the belt 34 is compressed due to the pressure between the drum 31 and the nip roll 33 its outer surface 35 tends to remain expanded to some extent even after it passes the center of the nip 38 and normally would contract as it starts to follow its concave path around the drum 31. However, as soon as the expanding influence of the nip is passed, the outer surface 35 of the belt contracts as the belt approaches its normal thickness and completes passage from its convex path around the nip roll 33 to its concave path around the drum 31.

As indicated in connection in FIG. 1, the surface 32 of the drum 31 is quite smooth, i.e., polished metal, and the drum is heated to further plasticize the web 40 and reduce the coefficient of friction between the drum and the web. In addition, the heated drum 31 serves to dry the web to some extent as it passes between the belt 34 and the drum after leaving the nip 38. Preferably, the interface between the web 40 and the surface 32 of the drum

is heated to a temperature of at least about the boiling point of water, i.e., 212° F., so as to generate moisture vapor. This moisture vapor both plasticizes the web 40 and creates a thin film or cushion of steam which materially reduces the coefficient of friction between the wet web and the heated drum. On the other hand, the web-contacting surface 35 of the belt preferably is relatively rough compared to that of the drum and the natural coefficient of friction of the belt is therefore greater than that of the drum. Thus, because of the natural differences between the coefficients of friction of the surface 32 of the drum and the surface 35 of the belt and because of the layer of steam between the web 40 and the drum, the paper web 40 tends to stick to the belt 34 and slip on the drum 31 with the result that when the outer surface 35 of the belt contracts, the web 40 is compacted horizontally or parallel to its median plane, in the direction of contraction of the belt surface. Since the belt contracts longitudinally, or in the machine direction, the web also is compacted longitudinally. During compaction the web 40 is confined between the belt 34 and the drum 31 by the pressure at the nip 38 and the tension on the belt 34 in such a way that the belt 34 exerts sufficient pressure with respect to the web faces to prevent substantial crinkling of the body of the web 40 and hold the web faces substantially flat and parallel to each other. Normally, for a belt approximately 1.25 inches thick, the nip force is in the neighborhood of about 150-240 pounds per inch of width and the tension on the belt is in the neighborhood of 120 pounds per inch of width. Normally, the web 40 is compacted longitudinally by about 10-25% of its original length by passing the web once through the apparatus of FIG. 4 in the manner described.

It is preferred that the impregnant be incorporated in the web 40 prior to compaction for the reasons indicated hereinbefore, particularly because higher compaction efficiencies can be attained. This improvement in efficiency of compaction which occurs when the web is impregnated prior to compaction may be explained on the theory that the impregnant exerts a "clutch action" upon the outer surface 35 of the contractile rubber belt 34, or grips the belt better, thereby increasing the frictional resistance of the web 40 to any movement relative to the outer belt surface 35.

For highest compaction efficiency, it is preferred that the temperature of the surface 32 of the drum be in the neighborhood of about 250° F. It also is preferred that the contractile belt 34 be cooled below the temperature of the drum particularly when the drum temperature is in the neighborhood of 250° F., to further increase the grip between the web 40 and the belt 34 and increase the effective like of the belt.

Referring to FIG. 4, a first cooling water spray nozzle 46 is positioned inside the belt 34, after the belt leaves the drum 31 in such a way as to direct a spray 47 of cooling water upon the underside of the belt before it reaches the tensioning roll 36. A second spray nozzle 48 is positioned outside the belt 34 opposite the tensioning roll 36 in such a way as to direct a spray 49 of cooling water upon the belt's outside surface 35. Finally, a bath 51 of cooling water is located in a trough 52 underneath the drum 31 and the bottom guide roll 37 is positioned to run partially submerged in the bath 51 so that the belt 34 passes through the bath and is cooled thereby. After leaving the bath 51 the belt 34 passes through the nip formed by a pair of squeeze rollers 52 which are adjusted to squeeze all but slight traces of the cooling water from the belt. When the surface of the drum 31 is maintained at about 250° F., the belt 34 preferably is maintained at about 170° F. by the cooling apparatus described. In this way, the belt has a much longer useful life than it would have if operated at the temperature of the drum.

After the compacted and partially dried web 40 leaves the surface 32 of the drum 31, it passes around a guide roller 53 and then down to a series of positioning rollers

54 which hold the web 40 out flat as it passes over a radiant heater 55 which completes the drying operation. The web 40, now in the form of a unified paper according to this invention, finally is led over another guide roller 56 and onto a wind up roll 57 on which it conveniently may be stored or supported for further processing.

FIGS. 5-7 are schematic drawings of longitudinal cross sections of portions of illustrative papers according to this invention before and after compaction. These cross sections are taken along lines extending longitudinally, or in the direction of compaction, of the web. Each of the papers, shown, contains the desired unifying amount of impregnant but for the sake of clarity the impregnant is shown only at the left end of each of the figures. The distribution of impregnant at the ends of the figures is typical of impregnant distribution throughout the body of the webs at the level of impregnation shown. In each figure, the enlargement is about 400 to 1. The dotted lines extending along the top and bottom faces of the webs represent the web faces, i.e., the surfaces of the webs as they would appear to the naked eye, and the center-lines designated M—P represent the median planes of the webs.

FIG. 5 depicts an impregnated but uncompacted flat starting web such as that designated F-61 Flat Impreg. Paper, in Example I hereinafter. This paper is formed from relatively unbeaten, softwood fibers 60 and is impregnated with particles or film portions 61 of a conventional rubbery latex, such as a unifying agent comprising a butadiene-acrylonitrile copolymer modified with a minor amount of a butadiene-styrene copolymer and a small amount of a phenolic resin, as will be described more fully hereinafter in Example I. The fibers 60 are substantially straight and possess only their natural curl and are oriented in the web predominantly parallel to the web faces 62 and flatly assembled in overlapping, crossing relation with one another extending in various directions parallel to the median plane M—P of the web. The fibers 60 are relatively long compared to the thickness of the web, i.e., averaging about 3.3 millimeters or 130 mils in length whereas the average thickness of the paper is about 4 or 4½ mils. It is obvious from this that the fibers 60 themselves lie flat in the web so that the overall orientation of a given fiber from end to end can only be at a slight or negligible angle to the faces 62 of the starting web.

FIG. 6 depicts a creped starting web formed from the same stock as the paper of FIG. 5 and impregnated with the same amount of the same impregnant 61. This paper is typical of that designated F-61 Crepe, Impreg. Paper in Example I hereinafter. As a result of creping the web has been opened up by movement of overlying fibers 60 in the web away from one another to increase the size of the voids or interstices 63 between the fibers. The web comprises large undulations, crepes or crinkles which are not clearly identifiable in FIG. 6 because of their size. In other words, the tip 64 of only one of these undulations appears in FIG. 6. Creped papers of this type are most open adjacent to the tips of these undulations, or crepes, and it is one of these most open portions of the web which is illustrated in FIG. 6. To show the whole of this undulation in the body of the web, itself, it would be necessary to have drawing about 3, 4, or more, times as long as that of FIG. 6. As explained in connection with the paper shown in FIG. 5, the fibers 60 in the paper, or web, of FIG. 6 are relatively long compared to the thickness of the web and flatly assembled in overlapping crossing relation with one another in the web.

FIG. 7 depicts the impregnated webs of FIG. 5 and FIG. 6, after compaction. This paper is typical of those designated F-61 Flat, Compacted I, Web, and F-61 Crepe, Compacted I, Web, in Example I hereinafter. During compaction in apparatus such as shown in FIG. 4, for example, the webs of FIGS. 5 and 6 are held between the belt 34 and the drum 31 and the belt 75 applies sufficient pressure to the web acting perpendicu-

larly with respect to the web faces 62 to prevent substantial crinkling of the web body and hold the web faces substantially flat while in contact with the drum and the belt.

The fibers 60 in the web of FIG. 7 are compressively distorted longitudinally, crowded and pushed together within the body of the web. The fibers, originally oriented primarily in the direction of compaction, i.e., longitudinally of the web, comprise kinks, or crimps, 65 which show in the plane of the cross section. This plane is perpendicular to the web faces 62 so that the fiber segments 66 forming these kinks are oriented at an angle to the web faces 62. It appears from FIG. 7 that a large proportion of the fiber segments 66 forming the kinks 65 are oriented at an angle to the web faces 62. As in FIGS. 5 and 6, the sectioned portions 60a of the fibers 60, represent fiber segments which are oriented, at least in part, laterally in the web, i.e., transversely of the direction of compaction.

Even though certain of the kinks 65 formed in the fibers as a result of compaction are reflected in small crenulations, i.e., very small and closely spaced humps 67 which may be visible to the naked eye, and adjacent depressions 67a in the surfaces of the web, the web body, itself, is not substantially crinkled. During compaction 20 the web body is densified, i.e., its fibers are brought closer together, and the web is maintained substantially flat. According to this invention, a large number of closely spaced kinks, or crimps 65, some of which are relatively tight, may be formed in the fibers originally extending 25 in the direction of compaction. For instance, normally about 100-400 kinks per inch are formed in the web in the fibers originally extending in the direction of compaction. This means that there may be about 12-48 kinks per fiber extending in this direction for papers formed from long fibered softwood pulps such as used in the free and open saturating papers of the prior art.

While in general the faces 62 of the web remain substantially flat, it should be noted that the top face 62, in FIG. 7, representing the face next to the compacting belt 34, is relatively rough or bumpy compared to the bottom face 62, representing that next to the drum 31, which is comparatively smooth. Thus, the faces 62 of the web tend to correspond somewhat with the respective surfaces of the belt 34 and the drum 31 with which they have been 45 in contact during compaction.

In unified papers according to this invention, as illustrated in FIG. 7, the fibers 60 are extensibly bonded together in their crowded and distorted state by the unifying material, or impregnant 61, in the web. The impregnant forms bonds between fiber segments 66 making up the kinks and adjacent fibers in the web, which bonds tend to retain the kinks so that the bonded fiber segments 66 tend to remain oriented at an angle to the web faces 62 and thereby resist delamination, or laminar separation of the fibers in the paper.

As indicated above, while compaction, according to this invention, does not result in substantial crinkling, i.e., the formation of relatively large undulations in the body of the web, itself, it may result in the formation of crenulations, or very small and closely spaced humps, in one or both of the surfaces of the web but normally in the web surface in contact with the relatively rough surface of the compacting belt. However, in general the web faces of the resulting unified compacted paper, according to this invention, are substantially flat and in all such papers the fibers are compressively distorted, crowded and pushed together within the body of the web and the fibers originally oriented primarily in the direction of compaction comprise a multiplicity of kinks, i.e., in the order of 100-400 kinks per inch in the web, with a large proportion of the fiber segments forming the kinks oriented at an angle to the web faces.

While the apparatus of FIG. 4 has been described in connection with the treatment of paper which is im-

pregnated prior to compaction, it also can be used for treatment of paper which is intended to be impregnated after compaction. Also, as mentioned hereinbefore and as will be described in the following examples, the starting web may be impregnated just prior to compaction so that some of the moisture included during impregnation may be used to plasticize the web and the steam chest may be eliminated.

The following additional examples are included to illustrate various embodiments of the process and of products according to this invention.

#### EXAMPLE I

A conventional saturating grade creped paper formed from relatively unbeaten, bleached, softwood, kraft fibers is impregnated with a conventional low modulus water based rubbery latex of the composition, set forth below, and having about 27% total solids, by passing the web through a bath of the impregnant composition and running the web through conventional squeeze rollers; and the impregnated web then is dried by conventional means. Impregnation is controlled so that the impregnant add-on, after drying, is about 25% by weight of the dry web.

| Aqueous impregnant composition                          |                                  |                 |
|---------------------------------------------------------|----------------------------------|-----------------|
| Material                                                | Trade name                       | Parts by weight |
| Butadiene-acrylonitrile (72:28) copolymer.              | Goodrich Hycar OR-25-----        | 762             |
| Butadiene-styrene (50:50) copolymer.                    | Dewey and Almy Darex 621L-----   | 182             |
| Butadiene-styrene (10:90) copolymer.                    | Dewey and Almy Darex 632L-----   | 83              |
| Heat curing phenol-formaldehyde resin.                  | Durez Plastics 14,798-----       | 13              |
| Tetra sodium salt of ethylene diamine tetraacetic acid. | Refined Products Permakleer #50. | 7               |
| Antioxidant-----                                        | Naugatuck Aminox Dispersion.     | 0.5             |
| Water-----                                              |                                  | 551             |

The impregnated web then is compacted in apparatus of the type shown in FIG. 4 essentially as described hereinbefore. The web is steamed to adjust its moisture content prior to compaction to about 15-20% by weight of the dry impregnated web and is compacted at a drum temperature of about 250° F. and a belt temperature of about 170° F. with a belt tension of about 120 pounds per inch of width and a nip force of about 230 pounds per inch of width to provide a degree of compaction of about 25% in one pass through the apparatus. The web then is dried as described in connection with FIG. 4 to provide a unified paper according to this invention. After compaction, the impregnant in the web is cured by subjecting the web to a temperature of 380° F. in an air circulating oven for about 1 minute.

The resulting unified paper possesses unexpectedly high delamination resistance for the small amount of impregnant it contains, extraordinary conformability, high flexibility, flatness, high tear strength, good tensile strength, and various other properties which make it particularly suitable for a backing for a pressure-sensitive adhesive masking tape as well as other uses. At only about 25% impregnation, according to this example, great cost savings are realized, yet superior results are obtained. The unexpectedly high delamination resistance of this paper and its importance will be described more fully hereinafter in connection with the data set forth in Table II. For purposes of comparison in analyzing delamination resistance, an additional sample is made and tested by compacting the starting web of this example without impregnant.

In other words, a control sample is prepared which is treated exactly the same as the above sample according to this invention except that the impregnation step is eliminated.

Full data for the original starting web, the control, the impregnated starting web and the resulting unified paper, according to this invention, designated "Compacted I. Web," on tensile strength, tear strength and elongation-to-break in the machine and cross directions; delamination resistance; caliper; basis weight; air porosity; apparent density and bulk; are given in Table I below under the heading F-61 Crepe.

A flat starting web the same as the above-described creped starting web, except for the fact that it is uncreped, is treated in the same way as the creped starting web to provide a unified paper according to this invention which possesses unexpectedly high delamination resistance, conformability, flexibility and elongation in the same order of magnitude as for the creped starting web, but higher tensile strength, lower tear strength and lower porosity. Full data for this impregnated and compacted flat starting web and its unimpregnated compacted control are given in Table I below under the heading F-61 Flat.

The data on tensile strength and percent elongation given in Table I are obtained by testing the papers in accordance with ASTM, Standard Test D-1000, the elongation figures being percent elongation-to-break, as mentioned above. Tear is determined by a modified Finch test of the type which has become standard in the paper masking tape industry. Delamination resistance is measured by preparing samples and testing them as described by Dunlap in "Some Factors Affecting Ply Adhesion in Latex Saturated Papers," appearing in Tappi, vol. 40, No. 8, August 1957, page 677. Caliper is measured in a conventional manner and basis weight is expressed in pounds per 320 square yards. Air porosity is expressed in seconds and represents the time in seconds needed for 400 cc. of air to pass through a paper web placed in a model 4110 Gurley Densometer with conditions controlled in accordance with Tappi Specification No. T-460, M-49. The figures given for apparent density represent the basis weight divided by thickness in mils, and bulk is expressed in cubic centimeters per gram as indicated.

Inspection of the delamination resistance given for the unified papers formed from the flat and creped starting webs of this example, shows the unexpectedly high delamination resistance of these papers compared with the delamination resistance of the impregnated starting webs, for example. The delamination resistance of the control, i.e., the compacted unimpregnated starting web, also is higher than the unimpregnated starting web. This, in itself, is surprising since prior art and prior experience indicate that compressive treatment of the web, if anything, may decrease delamination resistance. For instance, Cluett in United States Patent No. 2,624,245, which described a compacting operation similar to applicant's and essentially the same as disclosed in United States Patent No. 2,021,975 and Australian Patent No. 160,684, referred to hereinbefore, indicates that his compressing operation decreases the tensile strength of his paper. (Col. 6, lines 5-6 and lines 34-35.) All things being equal, a decrease in tensile strength of an unimpregnated web normally is associated with a decrease in delamination resistance. Thus the increased delamination resistance of the control samples is surprising in itself.

However, even if it is assumed that it would not be unexpected if the increased delamination resistance of a particular unified paper according to this invention merely equaled the sum of

(a) The delamination resistance of the impregnated uncompacted starting web, and

(b) The increment representing the increase in delamination resistance attributable to compaction alone,

i.e., the difference between the delamination resistances of the compacted control and the unimpregnated starting web, the delamination resistance of unified papers according to this invention is unexpected because it exceeds the above sum by an appreciable amount and therefore clearly exhibits synergism.

This now will be explained in more detail with particular references to Table II below. From theoretical considerations, it will be apparent that the total delamination resistance ( $D_T$ ) of any given "unified" and/or calendered or compacted paper may be represented by the equation:

$$D_T = D_P + D_C + D_I + K \quad (Equation I)$$

where:

$D_P$  = the delamination resistance of the untreated paper sheet.

$D_C$  = the increment in delamination resistance (over  $D_P$ ) contributed by the compacting step per se, in the absence of impregnation.

$D_I$  = the increment in delamination resistance (over  $D_P$ ) contributed by the impregnation step per se (in absence of any compacting step).

$K$  = a constant for any specific set of conditions.

Transposing the above equation to solve for the constant  $K$ :

$$K = D_T - D_P - D_C - D_I \quad (Equation II)$$

From Equation II it follows that:

(1) If  $K$  is zero, then the two operations mentioned above are purely additive or cumulative in their effect on the delamination resistance of the finished product;

(2) If  $K$  is a negative number, the two operations are antagonistic in their effect on delamination resistance of the finished product;

(3) If  $K$  is a positive number, the two operations are synergistic in their effect on delamination resistance of the finished product;

(4) In those instances where the two operations produce a synergistic (or an antagonistic) effect, the magnitude of the synergistic (or antagonistic) effect (expressed in terms of a percentage of the delamination resistance of an equivalently impregnated but uncompressed paper sheet) is given by the equation:

$$\text{Percent synergism (or antagonism)} = \frac{100 K}{D_P + D_I}$$

(5) If the basis of comparison is an equivalently compressed but unimpregnated sheet, the percent synergism (or antagonism) is given by the equation:

$$\text{Percent synergism (or antagonism)} = \frac{100 K}{D_P + D_C}$$

Table II tabulates the results obtained by applying the foregoing fundamental principles to some of the papers of Table I including the unified papers of this example.

## EXAMPLE II

Both the flat and creped unified papers of Example I are knife coated, in sheet form, with the following back-size composition, or release agent, diluted in a (50:50)

solution of toluene and methyl-ethyl-ketone to about 31 percent total solids:

*Backsize Composition*

| Material:                                     | Parts by weight | 5  |
|-----------------------------------------------|-----------------|----|
| Epoxy resin                                   | 6               |    |
| Polyvinyl chloride-acetate (87:13) copolymer  | 600             |    |
| High molecular weight polyester (plasticizer) | 210             |    |
| TiO <sub>2</sub>                              | 150             |    |
| 516 solution                                  | 240             | 10 |

*516 Solution*

| Material:             | Amount    |    |
|-----------------------|-----------|----|
| Sorbitan monostearate | lbs. 60   |    |
| Toluene diisocyanate  | lbs. 15   | 15 |
| Triethylamine         | ozs. 5    |    |
| Toluene               | gall. 31½ |    |

The coated paper is exposed to a temperature of 300° F. for approximately 1 minute to cure the backsize. The resulting backsize coating weights about 0.25 ounces per square yard. The opposite sides of the resulting coated sheets next are reverse roller coated, with the following pressure-sensitive adhesive mass dissolved in toluene to about 35% solids. The coated mass is dried and then cured by exposing the sheets to a temperature of 380° F. for approximately 1 minute. The resulting pressure-sensitive adhesive layer weighs about 2 ounces per square yard.

*Adhesive Mass*

| Material                                               | Trade name       | Parts by weight |    |
|--------------------------------------------------------|------------------|-----------------|----|
| Polyisoprene                                           | Pale Crepe #1    | 50.0            |    |
| Butadiene-styrene (77:23) copolymer                    | GRS 1022         | 50.0            |    |
| Diethylene glycol ester of dehydroabietic acid         |                  | 109.0           |    |
| p-Octylphenol formaldehyde                             | Amberol St 137   | 19.9            |    |
| Zinc oxide                                             | Protex           | 55.3            |    |
| 2,5 dinitro-allyl hydroquinone                         | Santovar A       | 2.2             | 40 |
| Tetra sodium salt of ethylene diamine tetraacetic acid | Refined Products | 1.6             |    |
| 2,6 dinitro-butyl-p-cresol                             | Permakleer #50   | 2.2             |    |
|                                                        | Ional            |                 |    |

Each of the resulting sheets, coated on one side with the backsize composition and on the other with the pressure-sensitive adhesive layer, then is slit into narrow widths by techniques which are conventional in the paper tape industry and the resulting pressure-sensitive adhesive tape is wound in successive helical convolutions upon itself in the form of a roll with the pressure-sensitive layer facing inwardly. A piece of tape recording to this example is shown in FIG. 3 wherein a layer 2 of a normally tacky and pressure-sensitive adhesive is applied to one side of a unified sheet 1 produced according to this invention and the backsize, not shown, is applied to the other side of the sheet 1.

The resulting rolls of tape formed from the flat and the creped starting webs of Example I are rapidly unwindable without any sign of delamination of the paper backing and are capable of being applied to smooth and rough surfaces and removed therefrom without delamination. After unwinding, both of these tapes possess a relatively high elongation, i.e., over 25% and are quite flexible. More importantly, perhaps, these tapes possess extraordinary ability to be conformed smoothly and easily to curved surfaces and other three-dimensional objects and to be smoothly applied in different shapes to flat surfaces. For instance, they may be applied in relatively sharp arcs to a flat surface without crinkling of one edge of tape and when used as a masking tape, give sharply defined paint lines without feathering at the edges of the tape. This is due mainly to the fact that the tape lies flat upon the surface to be painted and is not crinkled at its edges. The flatness of the tape backing also facil-

tates application of the tape in the first place and minimizes abrasion of the fingers of the worker applying it. In addition, these tapes are quite inexpensive, mainly due to the small amount of impregnant contained in the backing and the great variety of less expensive papers which may be used.

*EXAMPLE III*

A unified paper according to this invention is made by impregnating the creped starting web of Example I with the following solvent based impregnant composition, in the manner described in Example I, to provide an impregnant add-on after drying of about 22% by weight of the dry web. The following materials are dissolved in about 17 gallons of toluene:

*Solvent Impregnant*

| 20                                       | Material                       | Trade Name | Lbs. |
|------------------------------------------|--------------------------------|------------|------|
| Glycerol ester of hydrogenated resin.    | Hercules Staybelite Ester #10. | 24.4       |      |
| Zinc resinate                            | Newport Industries Zirex       | 2.25       |      |
| 2,6 dinitro-butyl-p-cresol               | Shell Ionol                    | 0.75       |      |
| p-Octyl phenol formaldehyde              | Rohm and Haas Amberol ST 137.  | 75.0       |      |
| 2,5 dinitro-allyl hydroquinone           | Monsanto Santovar A            | 0.75       |      |
| Nat. crude rubber in depolymerized form. | DPR-High Vis.                  | 70.5       |      |
|                                          | DPR Pigmented Compound.        | 9.0        |      |

The impregnated web then is compacted and dried as described in Example I. The paper then is cured by exposing it to a temperature of about 425° F. in an air circulating oven for a period of about 3 minutes to provide a unified paper according to this invention possessing unexpectedly high delamination resistance, extraordinary conformability, high flexibility, flatness, high tear strength, good tensile strength and the like as described in Example I. As in Example I, full data are given on these and other properties for the unimpregnated but compacted control, the impregnated web and the resulting unified paper in Table I below under the heading F-61 Crepe (Solvent Impreg.). Data for the starting web are the same as in Example I opposite F-61 Crepe. These data are obtained in the manner described in Example I. Data also are given for this paper in Table II on the synergistic increase in delamination resistance according to this invention.

The unified paper of this example is made into a tape wound upon itself in roll form by coating the paper with a backsize composition and an adhesive mass as described in Example II. The resulting pressure-sensitive adhesive tape is found to have all of the properties described in connection with the tape of Example II and therefore to possess particular advantages for use as a masking tape for curved surfaces and for masking difficult designs.

*EXAMPLE IV*

A unified paper according to this invention is formed from the same creped starting web and the same solvent based impregnant and in the manner described in Example III, but this time the starting web is compacted prior to incorporation of the impregnant, to provide a unified paper which possesses properties which are essentially equivalent to the properties of the unified paper of Example III. These properties are set forth in Table I under the heading F-61 Crepe (Solvent Impreg.) opposite "Impreg. Control." Again, synergism is demonstrated by corresponding data for this paper in Table II. A pressure-sensitive adhesive tape wound upon itself in roll form is fabricated as described in Examples II and III from the unified paper of this example with equivalent results.

TABLE I

| Ex. | Paper                        | Web                  | De-<br>gree<br>com-<br>pac-<br>tion | Lbs.<br>tensile |      | Lbs.<br>tear |       | Percent<br>elongation |      | Ozs.<br>delam.<br>res. | Caliper,<br>mils | Lbs.<br>basis<br>weight | Seconds<br>air<br>porosity | A.D.    | Bulk<br>cc./gm. |       |
|-----|------------------------------|----------------------|-------------------------------------|-----------------|------|--------------|-------|-----------------------|------|------------------------|------------------|-------------------------|----------------------------|---------|-----------------|-------|
|     |                              |                      |                                     | MD              | XD   | MD           | XD    | MD                    | XD   |                        |                  |                         |                            |         |                 |       |
| I   | F-61 flat kraft              | Starting web         |                                     | 27.5            | 11.0 | 96           | 101.3 | 2.2                   | 4.3  | 8.0                    | 3.5-4            | 31.2                    | 123.2                      | 8.3     | 2.13            |       |
|     |                              | Control              | 25                                  | 9.83            | 8.6  | 128          | 165.4 | 31.3                  | 5.1  | 13.5                   | 7.5-8.5          | 41.25                   | 224.5                      | 5.15    | 2.86            |       |
|     |                              | Impreg. starting web | 25                                  | 21.2            | 14.5 | 69.3         | 85.3  | 2.3                   | 10.5 | 27                     | 4-4.5            | 39.4                    | 489.6                      | -----   | -----           |       |
|     | F-61 crepe                   | Compacted I. web     | 25                                  | 25              | 24.8 | 16.2         | 96    | 138.7                 | 37   | 12.3                   | 50               | 6.5-7                   | 52.56                      | 1,069.2 | -----           | ----- |
|     |                              | Starting web         |                                     | 9.8             | 9.1  | 80           | 85.3  | 6.2                   | 4.0  | 18.0                   | 6-6.25           | 26.99                   | 12.9                       | 4.3     | 3.27            |       |
|     |                              | Control              | 23                                  | 6.5             | 7.83 | 149.3        | 122.6 | 33.3                  | 4.3  | 21.0                   | 5-6.5            | 35.95                   | 34.1                       | 6.31    | 2.33            |       |
| III | F-61 crepe (solvent impreg.) | Impreg. starting web | 27.5                                | 13.83           | 13.7 | 96           | 96    | 11.7                  | 7.08 | 34                     | 7.5-8.5          | 35.05                   | 16.02                      | -----   | -----           |       |
|     |                              | Compacted I. web     | 23                                  | 28              | 12.8 | 14.3         | 256   | 96                    | 44   | 9.25                   | 42               | 5-6                     | 44.5                       | 91.5    | -----           | ----- |
|     |                              | Control              | 23                                  | 6.5             | 7.83 | 149.3        | 122.6 | 33.3                  | 4.3  | 21.0                   | 5-6.5            | 35.95                   | 34.1                       | 6.31    | 2.33            |       |
| IV  | F-61 crepe (solvent impreg.) | Impreg. control      | 23                                  | 24              | 13.2 | 15           | 13.3  | 155.3                 | 35   | 7                      | 32               | 5.5-7                   | 42.34                      | 105.6   | -----           | ----- |
| V   | Patterson 556                | Starting web         |                                     | 24.6            | 17.0 | 64           | 53.3  | 1.67                  | 2.8  | 12.0                   | 2.75-3           | 26.8                    | 1,320                      | 9.3     | 1.49            |       |
| VI  | Patterson 556                | Control              | 24                                  | 13.7            | 13   | 85.3         | 106.6 | 31.1                  | 3.0  | 22.5                   | 7-8.5            | 35.4                    | 1,328                      | 7       | 3.16            |       |
|     |                              | Impreg. starting web | 20                                  | 14              | 14.2 | 69.3         | 64    | 1.3                   | 5    | 24                     | 3-3.25           | 31.76                   | 12,000                     | -----   | -----           |       |
|     |                              | Compacted I. web     | 25                                  | 20              | 17.8 | 16.3         | 64    | 80                    | 35.7 | 5.5                    | 50               | 7-9                     | 42.7                       | >12,000 | -----           | ----- |
|     |                              | Impreg. control      | 24                                  | 30.0            | 16.7 | 14.7         | 64    | 90.6                  | 17.5 | 4                      | 40               | 5.5-7.5                 | 38.3                       | >12,000 | -----           | ----- |
| VII | F-60 crepe                   | Starting web         |                                     | 11.6            | 5.3  | 74.6         | 96    | 9.5                   | 5.0  | 20.0                   | 7.5-7.9          | 28.8                    | 15.1                       | 3.5     | 4.01            |       |
|     |                              | Control              | 22.5                                | 9.08            | 5.5  | 117.3        | 122.6 | 34.6                  | 7.3  | 16                     | 5.5-6            | 36.87                   | 32.5                       | 6.47    | 2.31            |       |
| VII |                              | Impreg. starting web | 30.5                                | 13.6            | 9.0  | 98.3         | 96    | 10.3                  | 13   | 29.5                   | 8-8.5            | 37.6                    | 17.05                      | -----   | -----           |       |
|     |                              | Compacted I. web     | 21                                  | 30              | 15   | 11           | 112   | 112                   | 42.8 | 17.5                   | 42               | 5.5-6.5                 | 48.55                      | 67.05   | -----           | ----- |

TABLE II

| Example                          | Paper                        | Synergism in delamination resistance |        |    |     |    | Magnitude of synergistic effect, expressed as a percentage of delamination resistance of— |           |
|----------------------------------|------------------------------|--------------------------------------|--------|----|-----|----|-------------------------------------------------------------------------------------------|-----------|
|                                  |                              | Percent<br>impreg-<br>nation         | Ounces |    |     |    |                                                                                           |           |
|                                  |                              |                                      | DT     | DP | DC  | DR |                                                                                           |           |
| I                                | F-61 flat                    | 25                                   | 50     | 8  | 5.5 | 19 | 17.5                                                                                      | 65 129.5  |
| III—Impregnation then compaction | F-61 crepe                   | 28                                   | 42     | 18 | 3   | 16 | 5                                                                                         | 14.5 24   |
| IV—Compaction then impregnation  | F-61 crepe (solvent impreg.) | 22                                   | 35     | 18 | 3   | 3  | 11                                                                                        | 52.5 52.5 |
|                                  | do                           | 24                                   | 32     | 18 | 3   | 3  | 8                                                                                         | 38 38     |

## EXAMPLE V

A relatively dense flat paper starting web, such as sold under the name Patterson 556 by the Patterson Parchment Paper Co., and formed predominantly from moderately hydrated softwood fibers is impregnated with the aqueous impregnant composition of Example I and heated to dry the web as described in Example I, to provide an impregnant add-on of about 20% by weight of the dry web. The resulting impregnated sheet then is compacted as described in Example I at an initial moisture content of about 20% by weight of the dry web, dried and cured as described in Example I to provide a unified paper according to this invention. This paper possesses exceptionally good delamination resistance for the amount of impregnant it contains, i.e., 50 ounces delamination resistance for 20% impregnant. As in the papers of the preceding examples, conformability, elongation and flexibility are unusually good. Tensile strength is somewhat lower than that of the starting web but still very adequate, while the tear strength is substantially unchanged. The caliper of the unified paper is substantially increased over that of the starting web indicating that crenulations or humps along the surface of the paper are formed to a high degree. However, the faces of the paper are relatively flat and are capable of lying flat against any surface to which they may be applied. Thus, paper according to this example also is particularly suitable as a backing for a pressure-sensitive adhesive tape, such as a masking tape. Full data for paper according to this example are set forth in Table I under the heading Patterson 556, opposite "Compacted

45 I. Web." Similar data are given in this table for the unimpregnated starting web, the impregnated starting web, and for a control in the form of the compacted starting web.

## EXAMPLE VI

50 A unified paper according to this invention which is particularly suitable for a tape backing is formed from the same starting web, the same impregnant and in the same manner as described in Example V with the single exception that the web is compacted before it is impregnated. The resulting unified paper is substantially equivalent to that of Example V, except that its delamination resistance and elongation are not as high in proportion to the amount of impregnant added.

55 Full data for the paper of this example are set forth in Table I under Patterson 556, opposite "Impreg. Control."

## EXAMPLE VII

60 A saturating grade crepe paper formed from Canadian softwood kraft pulp with a high Alpha cellulose content and comprising a major percentage of fibers which have curls, or kinks, artificially imparted to them by a process similar to that described in United States Patent No. 2,516,384; is impregnated with the aqueous impregnant 65 of Example I and partially dried to bring the moisture content down to about 20%. The sheet, with this moisture content, then is compacted as described in Example I and finally completely dried and cured to provide a unified paper according to this invention having an impregnant add-on of approximately 30%. Detailed data for

this paper and its "control" are given in Table I under the heading F-60 Crepe. The resulting paper possesses excellent delamination resistance, conformability, elongation, flexibility, flatness, and is particularly suited for use as a paper masking tape backing.

## EXAMPLE VIII

A 400 yard length of a cheap (13¢/lb.) toweling grade, absorbent paper of 36# basis weight, produced by the

described. After compaction, the impregnant in sample "L" is cured as described in Example I.

Appreciably greater compaction is obtained with the impregnated sample "L" than with the unimpregnated sample "K" as indicated in the following Table C where in the figures under the columns headed "D," "B," "C," "V," "I," and "O" indicate drum and belt surface speed and paper speed at the points identified by the corresponding letters in FIG. 4:

TABLE C

| Sample                 | Operating conditions |                              |      |           |             |            | Percent compaction (Q) <sup>1</sup> | Percent efficiency of compaction (E) <sup>2</sup> |  |  |
|------------------------|----------------------|------------------------------|------|-----------|-------------|------------|-------------------------------------|---------------------------------------------------|--|--|
|                        | Drum surface speed D | Speed of belt surface 35 at— |      |           | Paper speed |            |                                     |                                                   |  |  |
|                        |                      | B                            | C    | V (calc.) | In (at I)   | Out (at O) |                                     |                                                   |  |  |
| K (unimpregnated)----- | 26.7                 | 22.3                         | 28.2 | 20.4      | 27.2        | 21.5       | 20.9                                | 74.6                                              |  |  |
| L (impregnated)-----   | 26.7                 | 22.3                         | 28.4 | 20.4      | 28.2        | 21.3       | 24.5                                | 87.5                                              |  |  |

<sup>1</sup> Percent actual compaction =  $(I-O)/I \times 100 = Q$ .

<sup>2</sup> Maximum theoretical compaction =  $(C-V)/C \times 100 = Z$ . Hence, percent efficiency of compaction =  $E = Q/Z \times 100 = Q/28 \times 100$ .

Brown Co. and sold primarily to the diary industry under the Brown trademark "Kowtowl," is wound upon a core and stored for about two weeks time at room temperature and coded "K" for identification purposes. Another 400 yard sample of the same starting web is impregnated with an aqueous latex to the extent of about 15% of its original weight as described in Example I; the latex composition used being as follows:

TABLE A

| Material                                                | Trade name                                  | Parts by weight |
|---------------------------------------------------------|---------------------------------------------|-----------------|
| Butadiene-acrylonitrile (72:28) copolymer.              | Goodrich "Hycar OR-25".                     | 3,320           |
| Butadiene-styrene (50:50) copolymer.                    | Naugatuck butadiene styrene copolymer 2001. | 3,320           |
| Heat curing phenol-formaldehyde resin.                  | Durez phenol-formaldehyde resin No. 14798.  | 81.5            |
| Tetra sodium salt of ethylene diamine tetraacetic acid. | Refined Products "Permaklear #50."          | 40              |
| Water.                                                  |                                             | 11,240          |

The impregnated 400 yard sample is dried and stored at room temperature for two to three weeks, wound upon a core and coded "L" for identification purposes.

Each of the foregoing 400 yard samples ("K" and "L") then is compacted as described in connection with FIG. 4 under the conditions set forth in Table B below:

TABLE B

|                           |                                             |  |
|---------------------------|---------------------------------------------|--|
| Nip roll:                 |                                             |  |
| Nip force -----           | Approximately 230 pounds per inch of width. |  |
| Diameter -----            | 6 inches.                                   |  |
| Rubber belt:              |                                             |  |
| Thickness -----           | 1.25 inches.                                |  |
| Hardness -----            | 55 Durometer.                               |  |
| Tension -----             | Approximately 120 pounds per inch.          |  |
| Heated roll:              |                                             |  |
| Diameter -----            | 23 inches.                                  |  |
| Surface speed -----       | 26.7 feet per second.                       |  |
| Surface temperature ----- | 250° F.                                     |  |

During both of these runs, the steam in the steam chamber is shut off in order to avoid possible differences in percent moisture pick-up. In other words, the two samples ("K" and "L") are plasticized with moisture during compacting only to the extent of their respective equilibrium moisture content after storage for two to three weeks at room temperature and atmospheric humidity as

From the data shown in Table C, in these directly comparable runs, it is clearly apparent that with the impregnated web (L), the degree of compaction is substantially higher than the degree of compaction attained with the unimpregnated web (K). It is also apparent that the compaction efficiency attained with the impregnated paper (L) is substantially greater (by 12.9%) than the compaction efficiency attained in processing the unimpregnated paper (K).

The improvement in efficiency of compaction attained with the impregnated web may be explained on the theory that the binder in the web exerts a "clutch action" upon the surface of the contractile rubber belt, increasing the frictional resistance of the web to any movement relative to the belt surface. Regardless, however, of the correctness of the suggested explanation, normally compaction of an impregnated paper under any given set of conditions in any given apparatus will produce a substantially higher degree of compaction and a higher efficiency of compaction than will be attained in processing an unimpregnated but otherwise identical paper in the same apparatus under substantially the same operating conditions.

The resulting unified paper according to this invention possesses remarkably improved delamination resistance for the cheap paper used and the relatively low amount of impregnant added and is extremely flexible and conformable, making it particularly suitable for a masking tape backing. The unified sheet of this example is coated on one side with the backsize composition of Example II and heated in the manner described in Example II to dry and cure the backsize. The resulting backsize layer weighs about 0.3 ounce per square yard. As in Example II, the opposite side of the sheet is coated with the following self-curing pressure-sensitive adhesive mass dissolved in toluene to about 33 percent solids to apply a pressure-sensitive adhesive layer weighing about 2.4 ounces per square yard:

## Self-Curing Mass

| 65 | Material                                               | Trade name                   | Parts by weight |
|----|--------------------------------------------------------|------------------------------|-----------------|
|    | Polyisoprene-----                                      | Polyisoprene pale crepe----- | 87.5            |
|    | Butadiene-styrene (77:23) copolymer.                   | GRS 1022-----                | 12.5            |
| 70 | Thermoplastic terpene tackifier (melt. point 315° C.). | Piccolyte S115-----          | 80.0            |
|    | Rosin modified maleic ester-----                       | Amberol M-88-----            | 10.0            |
|    | Aluminum hydrate-----                                  | Aluminum hydrate-----        | 50.0            |
|    | 2,5 diert butyl hydroquinone-----                      | Santovar A-----              | 2.0             |
|    | 2,6 diert butyl paracresol-----                        | Ionoil-----                  | 2.0             |
|    | Toluene diisocyanate-----                              | TDI-----                     | 2.5             |

The resulting pressure-sensitive adhesive sheet is slit

as described in Example II into rolls of tape wound in successive convolutions upon itself in the form of a roll with the pressure-sensitive layer facing inwardly. The tape rolls obtained do not delaminate when the tape is unwound rapidly from the roll and the tape exhibits extraordinary ability to conform to surfaces of various shapes. It also may be applied in sharp curves to flat surfaces without puckering at either edge of the tape. In other words the tape may be applied flat upon a flat surface in the form of a sharp curve. When used to mask a design of this type for spray painting, a sharply defined curved design is obtainable. The tape of this example is superior in this respect to competitive commercial tapes and yet is considerably less expensive due to the fact that it is made from a much cheaper starting web and much less impregnant, i.e., only about 15% by weight, is added to the backing.

#### EXAMPLE IX

A toweling grade "Kowtowl" web of the type described in Example VIII is impregnated with about 20% by weight of a high modulus, unplasticized, polyvinyl acetate resin in an aqueous dispersion containing about 15% solids. The impregnated web is compacted and cured as described in Examples I and VIII to provide a unified paper according to this invention with decidedly improved delamination resistance as indicated below:

| Paper:                | Delamination resistance (ozs.) |
|-----------------------|--------------------------------|
| Starting web          | 8                              |
| Impregnated web       | 16.9                           |
| Compacted impreg. web | 26.4                           |

The unified paper of this example is made into a pressure-sensitive masking tape in the manner described in Example VIII. The resulting tape is extremely flexible and conformable despite the high modulus impregnant employed and yet possesses improved firmness which facilitates handling and application of the tape to surfaces to be masked. There is no sign of delamination of the backing when the tape is unrolled and the tape is capable of conforming to surfaces of various shapes and being applied flat to define curved lines without puckering at the edges of the tape as described in Example VIII.

#### EXAMPLE X

The same "Kowtowl" starting web is impregnated as described in Example VIII using high modulus material of the following composition diluted to about 20 percent total solids by the addition of water.

##### High Modulus Impregnant

| Material                                                | Trade name              | Percent solids | Parts by weight |
|---------------------------------------------------------|-------------------------|----------------|-----------------|
| Butadiene-styrene acrylic acid (59:40:1)                | Lotol 2752              | 48             | 3,162.0         |
| Heat curing phenol-formaldehyde resin                   | Durez 14,798            | 65             | 1,063.0         |
| Tetra sodium salt of ethylene diamine tetraacetic acid. | Permakleer 60           | 33             | 21.2            |
| Anti-oxidant                                            | Aminox dispersion       | 52             | 2.6             |
| Potassium polyacrylate                                  | Acrysol G.S. diluted to | 1.2            | 104.0           |

The impregnated web is dried as described in Example I so that about 20% solids by weight of the dry web are added. The web then is compacted and cured according to Examples I and VIII to provide a unified web having improved delamination resistance as indicated below:

| Paper:                    | Delamination resistance (ozs.) |
|---------------------------|--------------------------------|
| Impregnated web           | 18.4                           |
| Compacted impregnated web | 30.4                           |

The resulting paper is made into a masking tape as described in Examples VIII and IX which is extremely

flexible and conformable and yet possesses good firmness for ease of application. This is another example of how a high modulus impregnant improves the firmness of the backing without seriously detracting from its conformability.

#### EXAMPLE XI

An artificial leather according to this invention is made from a relatively unhydrated flat bleached sulfate paper about 20 mils thick and having a basis weight of about 162 lbs., by first impregnating the paper with a water based acrylic latex to add about 21% impregnant solids by weight of the dry web and then compacting the impregnated web as described in Example I. The acrylic latex is one sold by Rohm and Haas of Philadelphia under the name Rhoplex B-15 and is believed to be essentially an ethyl acrylate polymer with a small percent of an acrylic acid modification. The impregnant composition comprises Rhoplex B-15 diluted to 25% solids and modified by the addition of 0.5% (solids on solids) of tetra-sodium ethylene diamine tetraacetic acid.

The following values are obtained for delamination resistance:

| Paper:                                         | Delamination resistance (ozs.) |
|------------------------------------------------|--------------------------------|
| Starting web                                   | 17                             |
| Control (compacted unimpregnated starting web) | 36                             |
| Impregnated web                                | 42                             |
| Compacted impregnated web                      | 67                             |

The resulting artificial leather possesses unexpectedly high delamination resistance, i.e., 67 ozs. and when flexed retains its integrity and does not blister or split. It also is free from fiber picking, i.e., the fibers are unified and are not easily removed from the web, accidentally or otherwise. This paper also is unusually soft and pliable and therefore adapted to be substituted for leather in many applications.

#### EXAMPLE XII

The starting web of Example V is treated as described in Example V except that the acrylate impregnant of Example XI is substituted for the impregnant composition of Example I with results very similar to those of Example V. Values obtained for delamination resistance are given below:

| Paper:                                         | Delamination resistance (ozs.) |
|------------------------------------------------|--------------------------------|
| Starting web                                   | 16                             |
| Control (compacted unimpregnated starting web) | 32                             |
| Impregnated web                                | 24                             |
| Compacted impregnated web                      | 48                             |

The resulting paper according to this invention is capable of many uses but is particularly suited for use as a tape backing because of its unexpectedly high delamination resistance and its extraordinary conformability.

#### EXAMPLE XIII

A flat moderately hydrated paper having a basis weight of about 32 lbs. and being about 4.6 mils thick and formed from bleached kraft softwood pulp is impregnated with an aqueous impregnant composition comprising about 30% of the following solids:

| Material:                                      | Parts |
|------------------------------------------------|-------|
| Buna N latex (33 acrylonitrile 67 butadiene)   | 88.4  |
| Tetra sodium ethylene diamine tetraacetic acid | 0.4   |
| Red pigments                                   | 11.2  |

The percent impregnation, i.e., add-on, is about 50% by weight of the dry starting web. The impregnated web is compacted as described in connection with FIG. 4 by adjusting its moisture content to about 15% by weight of the web and then passing the web through the com-

pacting unit to achieve a total degree of compaction of about 20% without substantially increasing the thickness of the web. The resulting paper according to this invention has improved flexibility, tear strength, and delamination resistance.

The unified paper of this example then is made into a sandpaper. First, one of its sides is coated with a barrier coat comprising a polyvinyl chloride resin plasticized with a copolymer of butadiene and acrylonitrile, and then a binder coat based upon a phenol-formaldehyde resin is applied to the barrier layer. The binder coat is several times thicker than the barrier coat and sand granules are applied to the paper by partially imbedding them in the wet binder coat. After drying the binder coat, a conventional sand size next is applied over the binder layer to provide a sandpaper according to this invention which possesses superior flexibility, tear strength and crack resistance.

#### EXAMPLE XIV

A rope paper of cylinder machine manufacture of 18 lbs. raw weight (24 x 36 x 480) is compressed to 65% of its original length by treatment in a laboratory adaption of the equipment described hereinabove and illustrated in the drawings.

An untreated sample of the paper showed the following characteristics:

|                       |                                                         |
|-----------------------|---------------------------------------------------------|
| M.D. tensile strength | 24 lbs./in.                                             |
| Caliper               | .002 inch.                                              |
| Gurley density        | 45 sec. (2 ply 400 cc.) 5 oz.<br>cylinder 1/4" opening. |

The above treated samples show M.D. tensile strength of 8 lbs./in.

|                |                                                         |
|----------------|---------------------------------------------------------|
| Caliper        | .0045 inch.                                             |
| Gurley density | 25 sec. (2 ply 400 cc.) 5 oz.<br>cylinder 1/4" opening. |

Samples of treated and untreated paper are impregnated in an aqueous colloidal dispersion of 33% total solids comprising as the dispersed phase:

|                                                                                                                                                                                                          |
|----------------------------------------------------------------------------------------------------------------------------------------------------------------------------------------------------------|
| 66% by weight of a copolymer of butadiene and acrylonitrile in the ratio of 75 parts butadiene to 25 parts of acrylonitrile emulsion polymerized in the presence of a fatty acid soap to a Mooney of 40. |
| 33.5% by weight of a copolymer of butadiene and styrene emulsion polymerized to a Mooney of 35.                                                                                                          |

0.5% of polymer solids of an antioxidant for the rubber.

Tests on the treated paper and on a control saturated to 100% by weight of solids of the above latex mixture show:

|                                 |           |
|---------------------------------|-----------|
| Compressed:                     | Control   |
| Tensile, 24.7#/in.              | 28.6#/in. |
| Delamination resistance, 100+oz | 60 oz.    |

#### EXAMPLE XV

A flat kraft paper of 38 lbs. basis weight (24 x 36 x 480) of the following characteristics:

|                |      |     |
|----------------|------|-----|
| M.D. tensile   | lbs. | 21  |
| Gurley density | sec. | 100 |

cannot be impregnated in the untreated state. After treatment by longitudinal compression to the extent of reduction in length of 10%, the sheet can be saturated.

Physical properties of the treated sheet are:

|                |             |
|----------------|-------------|
| M.D. tensile   | 10 lbs./in. |
| Gurley density | 52 sec.     |

Physical properties of the treated sheets saturated to the extent of 80% of the raw weight with the latex mixture described in Example I are:

|                         |                   |
|-------------------------|-------------------|
| M.D. tensile            | 22.5 lbs./in.     |
| M.D. elongation         | 14.8% elongation. |
| Delamination resistance | 35 oz.            |

The delamination resistance of the control sheet is only 20 ounces due to the poor impregnation thereof.

#### EXAMPLE XVI

5 A rope paper of cylinder machine manufacture of 30 lbs. basis weight (24 x 36 x 480) is compressed in the cross machine direction in a laboratory adaption of the equipment shown in the drawings. One sample of the sheet is passed through the compression machine once and another sample twice.

10 Both samples and a control are impregnated in an aqueous colloidal dispersion of 33% total solids comprising as the dispersed phase:

|                                                                                                                                                                                                               |
|---------------------------------------------------------------------------------------------------------------------------------------------------------------------------------------------------------------|
| 75 parts by weight of a copolymer of butadiene and acrylonitrile in the ratio of 75 parts butadiene to 25 parts of acrylonitrile emulsion polymerized in the presence of a fatty acid soap to a Mooney of 40. |
| 25 parts by weight of a copolymer of butadiene and styrene emulsion polymerized to a Mooney of 35.                                                                                                            |

15 The impregnated samples then are dried and heated at 380° F. for 1 minute in a circulating air oven. Tests on the compressed samples and the control give the following results:

|                           |                         |
|---------------------------|-------------------------|
| 20 Sample:                | Delamination resistance |
| Control                   | ounces 56               |
| 1 pass compression sample | do 79                   |
| 2 pass compression sample | do 133                  |

25 Cellulosic fibers of various sizes and shapes and of various conditions of hydration may be used in forming papers according to this invention. Typically, the starting web may comprise a major proportion of softwood kraft pulp preferably bleached or semi-bleached and slightly to moderately hydrated. Other cellulosic fibers such as rope fibers may be used as the major constituent and other fibers including hardwood fibers and even certain non-cellulosic fibers may be used as the minor constituent of the starting web in papers according to this invention. As mentioned hereinbefore, the starting web may be formed from fibers which are substantially straight and possess only natural curl or it may include a substantial proportion of fibers to which a substantial amount of curl or crimp has been imparted prior to web formation.

30 35 40 45 50 55 60 65 70 75 80 A variety of materials may be used as the impregnant, or unifying agent, for bonding the fibers in unified papers according to this invention. The term "unified papers" means primarily papers possessing increased resistance to splitting but is intended to also include increased resistance to fiber removal by spot picking or surface abrasion. Similarly, a "unifying amount" of the impregnant means that amount which prevents the paper from delaminating under normal conditions of use. These unifying materials may be classified generally as nonvolatile extensible polymers, extensible polymeric fiber bonding agents, elastomeric fiber bonding agents, or the like, and may be applied from water or from solvent based systems such as those based on volatile organic solvents, depending upon the material. They also may be classified as high and low modulus impregnants, both of which may be used in making papers according to this invention, as described hereinbefore.

75 80 85 90 95 The high modulus impregnants or polymers are in fact preferred at low levels of impregnation, i.e., about 10-30% by weight of the dry web. These high modulus materials, in the transition range of viscoelastic behavior, as described hereinbefore, include polyvinyl acetate polymers and copolymers, high styrene copolymers, such as high styrene (60-90% styrene) butadiene-styrene copolymers, polymethacrylate esters, polyvinyl alcohol, polyvinyl chloride, polyvinylidene chloride, polyvinyl acetals, polyurethanes, polyesters, and the like.

90 95 100 Suitable high modulus impregnants may be compounded by adding large amounts of modifying resins in conventional low modulus elastomer systems. For instance,

large amounts of heat curing phenolic resins may be used with chloroprene, isoprene, butadiene-styrene, butadiene-acrylonitrile or alkyl acrylate ester polymers and copolymers in such systems. Polyisocyanates and blocked polyisocyanates also may be used in the impregnant to increase the strength and modulus of the impregnant and to improve the bond between the polymer and the paper fibers.

Conventional low modulus extensible polymers also are suitable as impregnants in this invention. These include natural rubbers; diene polymers and copolymers such as: butadiene, isoprene and chloroprene polymers; copolymers of these materials with styrene, acrylonitrile, acrylamide, acrylic or methacrylic acids, acrylic or methacrylic acid esters; isobutylene polymers and copolymers; alkyl acrylate ester polymers and copolymers; polyvinyl ethers; glue-glycerine; and the like.

As mentioned hereinbefore the order of impregnation and compaction may be reversed although it is preferred to add the impregnant before compaction, and in certain cases it may be advantageous to perform impregnation and compaction in more than two steps. Another modification of the invention involves deposition of the unifying agent on the fibers prior to sheet formation. This prior treatment of the fibers with the bonding agent may be carried out by means of any of the known beater impregnation techniques and is most advantageously used when the compression mechanism is set up in connection with a paper machine. However, the principle may be modified by drying and rewetting the beater impregnated paper; or the paper, of suitable moisture content, may be stored in a moist condition and compressed after a convenient time interval. The fiber bonding materials applicable in this modification are limited to those which can be deposited by beater impregnation. The quantities of fiber bonding agent relative to fiber are limited naturally to the highest quantity which can be deposited onto the fibers. Usually somewhat less than the maximum quantity which can be deposited will make paper machine operation easier and result in an equal or superior final product. The lower limit may be determined only by evaluation of the final product for the use intended.

As indicated heretofore, the unified papers of this invention are particularly useful as backings for pressure-sensitive adhesive tapes. The paper backing may be coated in a suitable manner with a suitable adhesive mass to form a new and improved adhesive tape. The adhesive mass itself may be any of the conventional normally non-tacky solvent-activated, or normally tacky and pressure-sensitive adhesive masses that are so well known in the prior art. Most of the commonly used pressure-sensitive adhesives are based on relatively non-polar elastomers such as natural rubber, polyisoprene and the vulcanizable elastomeric copolymers and interpolymers of at least 40 percent butadiene and at least 10 percent styrene. Such an adhesive mass may be especially compounded, copolymerized or interpolymerized to have the desired degree of adhesiveness in absence of additional tackifiers. Or, alternatively, any of the conventional tackifiers may be used such as rosin, hydrogenated rosin, dehydrogenated rosin, the glycols and glycerides of any of these resinous materials, polyterpenes, coumarone indene resins, polyalkyl styrenes, oil-soluble aldehyde resins, or any other desired tackifier in any of the proportions that are so well known in the art. The adhesive mass may be free of an inert filler or may contain inert filler such as zinc oxide, magnesium carbonate, calcium carbonate, lead oxide, clay, titanium dioxide, aluminum, hydrated alumina, silica or any of the other conventional fillers for normally tacky and pressure-sensitive adhesives. Other ingredients such as anti-oxidants or heat stabilizers, dyes or pigments may be present or absent depending upon the particular desired use for the adhesive sheet. Typical normally tacky and pressure-sensitive adhesive masses are disclosed in Johnson & Johnson's British Patent No.

611,211 issued October 1948; in Nelson's United States Patent No. 2,415,901 issued February 18, 1949; in Pripke's United States Patent No. 2,405,926 issued August 13, 1946; in Buckley's United States Patent No. 2,397,774 issued April 2, 1946; and in many other patents. Exemplary of suitable normally non-tacky adhesives are conventional water-activatable glue adhesives, organic solvent-activated resinous adhesives such as those based upon vinyl chloride polymers, etc.

10 If desired, a priming coating may be interposed between the impregnated paper backing and the adhesive mass in order to secure improved adhesion of these two laminae. Any suitable priming coatings may be employed as, for example, those disclosed in the United States patent to Morris, No. 2,424,996. For ease in unrolling the tape, it is sometimes desirable to provide upon the surface of the backing, opposite that to which the adhesive mass is applied, a coating which decreases the adhesion of the adhesive mass to the face surface of the pressure-sensitive adhesive tape. Any suitable conventional release coating for such products may be employed as, for example, a lacquer, a surface-active material of the type disclosed in the United States patent to Collins, No. 2,913,355, etc.

15 When the paper backing for pressure-sensitive adhesive tape according to this invention is formed by compacting the paper horizontally by at least about 5% to about 40% of its length, the tape resulting from processing as described above normally will be extensible to the extent of at least about 5% to about 40% in length when stretched lengthwise.

20 25 An example of such a tape according to this invention is shown in FIG. 3 wherein a coating 2 of a normally tacky and pressure-sensitive adhesive is applied to one side of a unified sheet produced in accordance with this invention, which sheet forms the backing of the tape.

25 30 Having now described the invention in specific detail and exemplified the manner in which it may be carried into practice, it will be readily apparent to those skilled in the art that innumerable variations, applications, modification, and extensions of the basic principles involved may be made without departing from its spirit or scope.

35 What is claimed is:

1. A pressure-sensitive adhesive masking tape comprising a unified paper backing coated on one surface thereof with a pressure-sensitive adhesive, said tape being wound in successive convolutions upon itself to form a roll from which it is rapidly unwindable without delamination of said paper backing, and when so unwound, is extensible to the extent of at least about 5% in length when stretched lengthwise; said unified paper backing being composed of distorted, longitudinally crowded cellulose fibers, bonded together by about 10-30% by weight of the dry fibers of a high modulus extensible polymeric unifying material distributed within the body of the backing to increase the firmness and delamination resistance of the backing, said unifying material being in the transition range of viscoelastic behavior; the fibers of said backing being distorted and longitudinally crowded by subjecting a starting web having an elongated web body composed of cellulose fibers and having two opposed web faces, while heated to a temperature sufficient to generate moisture vapor, simultaneously to (a) sufficient confining pressure, acting perpendicularly with respect to said web faces to prevent substantial crinkling of the web body, and (b) sufficient compacting force, acting longitudinally with respect to the length of said web (i) to cause the web fibers to be longitudinally distorted and forced closer together in changed orientation lengthwise within the web body and (ii) to cause the web body thereby to contract 40 in length by at least about 5%; whereby an inexpensive tape is provided characterized by (a) high resistance to delamination, (b) high conformability, and (c) good firmness.

45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 939

aterial, artificial leather and the like; said paper sheet comprising (a) cellulosic papermaking fibers that are compressively distorted, and crowded together within the body of said sheet and (b) an extensible, polymeric fiber-bonding agent, distributed substantially throughout the body of said sheet in unifying amount and in fiber-bonding relationship with said cellulosic fibers to bond said fibers in their distorted and crowded state; said unified, compacted paper sheet being formed by compaction of a paper starting web having a sheet-like web body composed essentially of cellulosic papermaking fibers, and a median plane lying generally between its web faces, by carrying out the following operations upon said starting web, to wit:

- (1) incorporating into said web a polymeric fiber-bonding agent in a proportion which is unifying after compaction, thereafter
- (2) subjecting said polymer-containing starting web, while plasticized with moisture and heated to a temperature sufficient to generate moisture vapor, simultaneously:
  - (a) sufficient compacting force, acting in a direction generally parallel to said median plane, substantially to contract the area of said web body and to distort and crowd said fibers closer together in changed orientation with respect to each other, within said web body between said faces; and
  - (b) sufficient confining force, acting in a direction generally perpendicular to said median plane, to prevent substantial crinkling of said web body during such compaction; and
- (3) drying said compacted web to bond the distorted fibers in their changed orientation.

3. A unified compacted paper according to claim 2, wherein the amount of the extensible polymeric fiber-bonding agent present is at least about 10% by weight of the dry web.

4. A unified compacted paper according to claim 3, wherein the amount of the extensible polymeric fiber-bonding agent present is not above about 50% by weight of the dry web and said fiber-bonding agent is in the transition range of viscoelastic behavior.

5. A unified, compacted paper sheet according to claim 2, wherein said starting web is creped.

6. A unified, compacted paper sheet according to claim 2, wherein said starting web is uncreped.

7. A relatively dense, unified, compacted paper sheet adapted to be used as a backing for adhesive tape, abrasive sheet material, artificial leather and the like; said paper sheet comprising (a) cellulosic papermaking fibers that are compressively distorted, crowded and pushed together within the body of said sheet and (b) an extensible polymeric fiber-bonding agent, distributed within the body of said sheet in unifying amount and in fiber-bonding relationship with said cellulosic fibers to bond said fibers in their distorted and crowded state; said distorted fibers being formed from a paper web composed of cellulosic papermaking fibers and having a web body between two opposed, substantially parallel web faces, by carrying out the following operations upon said paper web, to wit:
 

- (1) incorporating into said web a unifying proportion of said polymeric fiber-bonding agent dispersed in an aqueous vehicle; thereafter (2) simultaneously (a) applying force, acting perpendicularly with respect to said web faces, to prevent substantial crinkling of said polymer-containing web body and to maintain said web faces substantially parallel to each other, and (b) compacting the web in a direction parallel to said web faces while said polymer-containing web is plasticized with moisture and heated to a temperature sufficient to generate moisture vapor, thereby (i) to distort and crowd the web fibers together horizontally in changed orientation within the web body and (ii) to contract the area of the web by at least 5% to about 40%; and (3) drying said compacted web to bond the distorted fibers in their changed orientation; said unified compacted paper sheet being characterized by (a) high resistance to delamination and (b) substantial extensibility when stretched in a direction parallel to the direction of compaction.

5 by at least 5% to about 40%; and (3) drying said compacted web to bond the distorted fibers in their changed orientation; said unified compacted paper sheet being characterized by (a) high resistance to delamination and (b) substantial extensibility when stretched in a direction parallel to the direction of compaction.

8. A relatively dense, unified, compacted paper sheet adapted to be used as a backing for adhesive tape, abrasive sheet material, artificial leather and the like; said paper sheet comprising (a) cellulosic papermaking fibers that are compressively distorted, crowded, and pushed together within the body of said sheet and (b) an extensible, polymeric fiber-bonding agent, distributed within the body of said sheet in unifying amount and in fiber-bonding relationship with said cellulosic fibers to bond said fibers in their distorted and crowded state; said distorted fibers being formed from a paper web composed of cellulosic papermaking fibers and having a web body between two opposed, substantially parallel web faces, by carrying out the following operations upon said paper web, to wit:
 

- (1) incorporating into said web a unifying proportion of said polymeric fiber-bonding agent; thereafter (2) simultaneously (a) applying force, acting perpendicularly with respect to said web faces, to prevent substantial crinkling of said polymer-containing web body and to maintain said web faces substantially parallel to each other, and (b) compacting the web in a direction parallel to said web faces while said polymer-containing web is plasticized with moisture and heated to a temperature sufficient to generate moisture vapor, thereby (i) to distort and crowd the web fibers together horizontally in changed orientation within the web body and (ii) to contract the area of the web by at least 5% to about 40%; and (3) drying said compacted web to bond the distorted fibers in their changed orientation; said unified compacted paper sheet being characterized by (a) high resistance to delamination and (b) substantial extensibility when stretched in a direction parallel to the direction of compaction.

35 9. In the manufacture of a pressure-sensitive adhesive tape by forming a unified, extensible, elongated paper backing, coating one surface of said backing with a water insoluble, normally tacky and pressure-sensitive adhesive mass and winding the coated backing upon itself to form a roll of tape; that improvement which comprises forming said unified extensible paper backing by (a) impregnating a paper web having opposed, substantially parallel web faces and an elongated web body composed of cellulose fibers, with an aqueous dispersion of an extensible polymeric fiber-bonding agent in an amount sufficient substantially to increase the resistance of the dried web to delamination; (b) passing said impregnated web, while plasticized with moisture, between two moving surfaces, (i) one of said moving surfaces being a heated, inelastic, polished metal surface that, in cooperation with the moisture vapor generated during contact of the web therewith, offers relatively low frictional resistance to the movement of the web in contact therewith, (ii) the other of said moving surfaces being a contractile, yieldably supported, rubber surface that, in cooperation with said fiber-bonding agent, offers relatively high frictional resistance to the movement of the web in contact therewith; (c) maintaining said heated surface at a temperature sufficient to generate moisture vapor during contact of the moisture-plasticized web therewith and subsequently to cause at least partial drying of said web; (d) confining said web, while passing between said moving surfaces, under sufficient pressure, acting perpendicularly with respect to the web faces (i) to prevent substantial crinkling of the web body and (ii) to hold said web faces substantially parallel to each other while in contact with said moving surfaces; (e) simultaneously longitudinally contracting said contractile surface in a direction counter to the direction of movement of the confined web (i) to cause the web fibers, in the presence of said fiber-bonding agent

in the web body, to be longitudinally distorted and forced closer together in changed orientation lengthwise within the web body, and (ii) thereby to cause the web body to contract in length by at least from about 5% to about 40%; and (f) drying the contracted web, thereby to retain the distorted fibers extensibly bonded together in their changed orientation; whereby to obtain a roll of pressure-sensitive tape that is rapidly unwindable from the roll without delamination of said unified backing, and when so unwound, is extensible to the extent of at least about 5% to about 40% in length when stretched lengthwise.

10. In the manufacture of a unified, extensible cellulosic fibrous paper sheet adapted to be used as a backing for adhesive tape, abrasive sheet material, artificial leather and the like; that improvement which comprises: (1) incorporating in a cellulosic fibrous paper web a unifying proportion of an extensible polymer in fiber-bonding relationship with the cellulosic fibers thereof; thereafter (2) simultaneously (a) applying force, acting perpendicularly with respect to the principal surfaces of the web, to prevent crinkling of the body of the web, and maintain said principal web surfaces substantially parallel to each other and (b) compacting the web, horizontally with respect to the principal surfaces of the web, while said polymer-containing web is plasticized with moisture and heated to a temperature sufficient to generate moisture vapor, thereby (i) to distort and crowd the web fibers together horizontally in changed orientation within the body of the web and (ii) to contract the area of the web by at least about 5% to about 40%; and (3) drying the compacted web containing said extensible binder to internally bond the distorted fibers in their changed orientation; whereby to obtain a unified, compacted, internally bonded, cellulosic fibrous web characterized by (a) high resistance to delamination and (b) substantial extensibility when stretched in a direction parallel to its direction of compaction.

11. The improvement of claim 10 wherein said extensible polymer is incorporated in a cellulosic fibrous web by beater impregnation during web formation thereof.

12. The improvement of claim 10 wherein said extensible polymer is incorporated in a fibrous web by impregnating a preformed cellulosic fibrous web with said polymer dissolved in a volatile organic solvent.

13. An improvement of claim 10, wherein said web is plasticized during said compacting step by a moisture content not substantially greater than said web's equilibrium moisture content when stored at about room temperature at about 50% relative humidity.

14. In the manufacture of a unified, extensible cellulosic fibrous paper sheet adapted to be used as a backing for adhesive tape, abrasive sheet material, artificial leather and the like; that improvement which comprises: (1) incorporating in a paper web of papermaking cellulosic fibers a unifying proportion of an extensible polymer in fiber-bonding relationship with said cellulosic fibers by impregnation of said paper web with an aqueous dispersion of said polymer; thereafter (2) simultaneously (a) applying force, acting perpendicularly with respect to the principal surfaces of said paper web, to prevent substantial crinkling of the body of the web and to maintain said principal surfaces substantially parallel to each other, and (b) compacting said paper web, in a direction parallel to said principal surfaces, while said polymer-containing paper web is plasticized with moisture and heated to a temperature sufficient to generate moisture vapor thereby (i) to distort and crowd said cellulosic fibers horizontally together in changed orientation within the body of the paper web and (ii) to contract the area of the paper web by at least about 5% to about 40%; and (3) drying the polymer-containing compacted paper web to internally bond the distorted fibers in their changed orientation; whereby to obtain a unified compacted paper web characterized by (a) high resistance to delamination and (b)

substantial extensibility when stretched in a direction parallel to its direction of compaction.

15. A pressure-sensitive adhesive tape comprising a unified paper backing coated on one surface thereof with a normally tacky and pressure-sensitive adhesive, said tape being wound in successive convolutions upon itself to form a roll from which it is rapidly unwindable without delamination of said backing; said backing being composed of (a) paper-making cellulosic fibers that are compressively distorted and crowded together within the body of the backing, and (b) an extensible, polymeric, fiber-bonding agent, distributed substantially throughout the body of such backing in unifying amount and in fiber-bonding relationship with said fibers to bond said fibers together in their distorted and crowded state; said backing being formed by carrying out the following operations, to wit:

(1) providing a starting web comprising an open, porous paper web composed essentially of paper-making cellulosic fibers, said starting web having a sheet-like web body with a median plane lying generally between its web faces;

(2) subjecting said starting web, while plasticized with moisture and heated to a temperature sufficient to generate moisture vapor, simultaneously to:

(a) sufficient compacting force, acting in a direction generally parallel to said median plane, substantially to contract the area of said web body and to distort and crowd said fibers closer together in changed orientation with respect to each other, within said web body between said faces; and

(b) sufficient confining force, acting in a direction generally perpendicular to said median plane, to prevent substantial crinkling of said web body during such compaction;

thereby to produce a compacted intermediate web that is (i) nonunified, (ii) less absorbent than said starting web and (iii) structurally stable in the presence of moisture;

and (3) thereafter unifying said compacted intermediate web by impregnation with a fiber-bonding agent comprising an extensible polymer to distribute a unifying proportion of said fiber-bonding agent substantially throughout the body of said intermediate web, in fiber-bonding relationship with said distorted fibers and thereby to produce a compacted and unified web having a delamination resistance that is substantially greater than the delamination resistance of an uncompacted but otherwise identical impregnated web.

16. A pressure-sensitive adhesive tape according to claim 15, wherein the amount of the extensible polymeric fiber-bonding agent present is about 10-50% by weight of the dry web and said fiber-bonding agent is in the transition range of viscoelastic behavior.

17. A pressure-sensitive adhesive tape according to claim 15 wherein the starting web is formed from a slightly to moderately hydrated paper pulp.

18. A pressure-sensitive adhesive tape comprising a unified paper backing coated on one surface thereof with a normally tacky and pressure-sensitive adhesive, said tape being wound in successive convolutions upon itself to form a roll from which it is rapidly unwindable without delamination of said backing; said backing being composed of (a) paper-making cellulosic fibers that are compressively distorted and crowded together within the body of the backing, and (b) an extensible, polymeric, fiber-bonding agent, distributed substantially throughout the body of such backing in unifying amount and in fiber-bonding relationship with said fibers to bond said fibers together in their distorted and crowded state; said tape being formed by carrying out the following operations, to wit:

(1) providing a starting web comprising an open, porous paper web composed essentially of paper-making cellulosic fibers, said starting web having a sheet-

31

like web body with a median plane lying generally between its web faces;

(2) subjecting said starting web, while plasticized with moisture and heated to a temperature sufficient to generate moisture vapor, simultaneously to:

(a) sufficient compacting force, acting in a direction generally parallel to said median plane, substantially to contract the area of said web body and to distort and crowd said fibers closer together in changed orientation with respect to each other, within said web body between said faces; and

(b) sufficient confining force, acting in a direction generally perpendicular to said median plane, to prevent substantial crinkling of said web body during such compaction;

thereby to produce a compacted intermediate web that is (i) nonunified, (ii) less absorbent than said starting web and (iii) structurally stable in the presence of moisture;

(3) thereafter unifying said compacted intermediate web by impregnation with a fiber-bonding agent comprising an extensible polymer to distribute a unifying proportion of said fiber-bonding agent substantially throughout the body of said intermediate web, in fiber-bonding relationship with said distorted fibers and thereby to produce a compacted and unified web having a delamination resistance that is substantially greater than the delamination resistance of an uncompacted but otherwise identical impregnated web;

(4) coating one surface of said compacted, unified paper web with a pressure-sensitive adhesive mass; and

(5) winding said coated web in successive convolutions

32

upon itself to form a roll of pressure-sensitive adhesive tape that is rapidly unwindable from said roll without delamination of said compacted, unified and coated web.

5 19. The product of claim 18 wherein said web, during the application of said compacting force, is contracted in area by at least 5% to about 40%.

20. The product of claim 19 wherein said unifying operation is carried out by impregnating said compacted intermediate with said fiber-bonding agent dispersed in a volatile organic solvent and thereafter evaporating said volatile solvent.

21. The product of claim 19 wherein said unifying operation is carried out by impregnating said compacted intermediate with said fiber-bonding agent dispersed in an aqueous vehicle and thereafter evaporating said aqueous vehicle.

#### References Cited in the file of this patent

##### UNITED STATES PATENTS

|           |                 |                |
|-----------|-----------------|----------------|
| 2,021,975 | Wrigley et al.  | Nov. 26, 1946  |
| 2,410,078 | Kellgren        | Oct. 29, 1946  |
| 2,415,901 | Nelson et al.   | Feb. 18, 1947  |
| 2,450,083 | Donaldson       | Sept. 28, 1948 |
| 2,624,245 | Cluett          | Jan. 6, 1953   |
| 2,633,430 | Kellgren et al. | Mar. 31, 1953  |
| 2,666,699 | McQuiston       | Jan. 19, 1954  |
| 2,726,967 | Eger et al.     | Dec. 13, 1955  |
| 2,728,687 | Huerre          | Dec. 27, 1955  |
| 2,768,092 | Lawrence        | Oct. 23, 1956  |
| 2,848,355 | Bartell         | Aug. 19, 1958  |

UNITED STATES PATENT OFFICE  
CERTIFICATE OF CORRECTION

Patent No. 3,055,496

September 25, 1962

Isaac R. Dunlap

It is hereby certified that error appears in the above numbered patent requiring correction and that the said Letters Patent should read as corrected below.

Column 2, line 10, strike out "to"; column 3, line 73, for "exhaustive" read -- extensive --; column 9, line 52, for "like" read -- life --; column 10, line 62, after "have" insert -- a --; column 29, line 22, before "crinkling" insert -- substantial --.

Signed and sealed this 5th day of February 1963.

(SEAL)

Attest:

ERNEST W. SWIDER  
Attesting Officer

DAVID L. LADD  
Commissioner of Patents